

Aug. 25, 1953

G. E. REESE ET AL

2,650,188

PREPARATION OF LUBRICATING OIL

Filed Nov. 1, 1949

3 Sheets-Sheet 1

Fig. 1



INVENTORS.  
GEORGE E. REESE  
BY JOHN L. LARKIN

Burke and Hardin  
ATTORNEYS

Aug. 25, 1953

G. E. REESE ET AL

2,650,188

PREPARATION OF LUBRICATING OIL

Filed Nov. 1, 1949

3 Sheets-Sheet 2



INVENTORS  
GEORGE E. REESE  
JOHN L. LARKIN  
BY

Bassett and Harding  
ATTORNEYS

Aug. 25, 1953

G. E. REESE ET AL.

2,650,188

PREPARATION OF LUBRICATING OIL

Filed Nov. 1, 1949

3 Sheets-Sheet 3



INVENTORS  
GEORGE E. REESE  
JOHN L. LARKIN

BY

Burke and Harding

ATTORNEYS

Patented Aug. 25, 1953

2,650,188

# UNITED STATES PATENT OFFICE

2,650,188

## PREPARATION OF LUBRICATING OIL

George E. Reese, Wallingford, and John L. Larkin, Ridley Park, Pa., assignors to Sun Oil Company, Philadelphia, Pa., a corporation of New Jersey

Application November 1, 1949, Serial No. 124,892

4 Claims. (Cl. 196—41)

**1** This invention relates to the preparation of lubricating oil from naphthenic base crude petroleum by distillation.

In obtaining lubricating oil fractions from crude petroleum it is customary practice to subject the crude oil to a primary distillation or topping operation, usually conducted at approximately atmospheric pressure, in which the lighter hydrocarbon fractions such as gasoline, kerosene and gas oil are removed. The resulting mazout or residuum fraction is then treated with aqueous caustic soda to neutralize acidic constituents, after which it is subjected to vacuum distillation to obtain lubricating oil as distillate. Usually the vacuum distillation is carried out in such manner as to obtain a plurality of lubricating oil cuts of different boiling range and viscosity, which subsequently may be blended as required to obtain various grades of commercial products.

In practicing such prior art process with naphthenic base crude as the starting material, it has been found that the distillate lubricating oil fractions may have certain undesirable characteristics which reduce their value as commercial products. One such characteristic is lack of color stability, the oils tending to darken more or less readily upon standing. Improvement may be effected in color stability by subsequent treatment of the oils with sulfuric acid and clay, but this entails considerable additional expense in their preparation. Another characteristic which, while not affecting the lubricating quality of the products, is considered important because it affects their salability is the bloom or appearance of the oils by reflected light. Distillate oils from naphthenic base crudes tend to have a bluish bloom which imparts a more or less dark appearance and reduces market value, in contrast to the greenish bloom and brighter appearance of distillate oils derived from crudes of the Pennsylvania type.

We have now found that the color stability and bloom characteristics of oils derived from naphthenic base crudes can be distinctly improved by reacting charge material, prior to the vacuum distillation step, not only with caustic soda but also with ammonia. The resulting distillates from the vacuum distillation will have more stable colors and a greener bloom imparting a brighter appearance. In order to secure these results, the amounts of both caustic soda and ammonia used should exceed certain minimum values as hereinafter more fully specified.

The present invention thus provides a process for producing from naphthenic base crudes dis-

**2** tillate lubricating oils having improved bloom and color stability characteristics. According to the invention naphthenic base stock containing lubricating oil hydrocarbons is reacted, prior to vacuum distillation, with ammonia in the presence of caustic soda. This may be done in several ways as follows:

- (1) By subjecting the crude petroleum first to a topping operation, then treating the resulting mazout with aqueous caustic soda and with ammonia and then vacuum distilling;
- (2) By first treating the crude with aqueous caustic soda and with ammonia, then topping the crude and vacuum distilling the mazout; and
- (3) By first treating the crude with aqueous caustic soda, then topping, then treating the mazout with ammonia and finally vacuum distilling.

**10** 20 Combinations of these procedures, wherein part of the ammonia and caustic soda or part of each is added prior to the topping operation and the remainder is added to the mazout, may also be used.

**25** It is to be noted that the invention does not include the sequence of steps of treating the crude with ammonia alone, then topping, then treating with caustic soda alone and finally vacuum distilling. In such procedure the ammonia is driven off during the primary distillation or topping operation, so that none is present at the time when the mazout is treated with caustic soda. While the process may be practiced in several different ways as specified above, it is always important that caustic soda be present in the stock at the time it is reacted with the ammonia.

**40** In order to secure substantial improvement in the foregoing characteristics of the lubricating oil distillates, it is also important that the amount of aqueous caustic soda used be at least equivalent to 1.2 lbs. NaOH per bbl. of mazout resulting from the primary distillation and that the ammonia be added in an amount of at least 0.1 lb. NH<sub>3</sub> per bbl. of mazout. These minimum amounts apply regardless of which of the permissible sequence of steps is utilized in practicing the invention. Preferably the caustic soda and ammonia should be employed in amounts exceeding, respectively, 1.5 lbs. NaOH and 0.2 lb. NH<sub>3</sub> per bbl. of mazout. The proportions to be used for securing results desired for commercial operation may vary considerably for different naphthenic base crudes, but as a general rule the desired improvement will be obtained without exceeding 5.0 lbs. NaOH and 0.5 lb. NH<sub>3</sub> per bbl.

of mazout. Selection of preferable proportions of caustic soda to use for different crude stocks may be based upon the free NaOH content of the mazout which is to be vacuum distilled. It is generally desirable that the amount of caustic soda employed be sufficient to impart a free NaOH content of at least about 0.10% to the mazout. A still higher free NaOH content, such as 0.15-0.30%, may aid in securing maximum improvement in color stability.

While the strength of the caustic soda solution is not of critical significance as long as the required amount of NaOH is supplied, it is preferred to employ a relatively concentrated solution such as caustic soda of 38-50° Bé., so that the amount of water evaporated during the operation will be small. The ammonia may be added either as a gas or as aqueous ammonia. Suitable means should be provided for intimately contacting the treating agents with the hydrocarbon stocks to secure efficient utilization of the treating agents added.

Several ways in which the present invention may be practiced are illustrated diagrammatically in the accompanying drawings in Figs. 1-3. In Fig. 1 naphthenic base crude petroleum is subjected to a primary distillation in distillation zone 10 to remove hydrocarbons boiling below the lubricating oil range. The hot residuum or mazout then passes to treating zone 11 wherein it is 15 intimately contacted with caustic soda and ammonia in the amounts required. Either the caustic soda or the ammonia may be added first, or the two may be introduced into the mazout simultaneously. After such treatment any sludge formed may, if desired, be separated from the treated oil. The treated mazout is then subjected to distillation under essentially non-cracking conditions in vacuum distillation zone 12 to obtain the desired lubricating oil as distillate. Constituents containing inorganic matter resulting from the addition of caustic soda, such as sodium naphthenates, remain in the heavy residuum. During the vacuum distillation additional quantities of ammonia advantageously may be introduced to aid in securing the desired improvement in characteristics of the lubricating oil produced.

Referring to Fig. 2, the crude petroleum is first treated with caustic soda and ammonia in the required amounts in treating zone 13. Here, again, either treating agent may be added first or they may be introduced simultaneously. The crude is then subjected to primary distillation in zone 14 and the resulting mazout is vacuum distilled, with or without further introduction of ammonia, in zone 15.

The sequence of steps illustrated by Fig. 3 comprise first treating the crude with caustic soda in zone 16, topping in primary distillation zone 17, then treating the mazout with ammonia in zone 18 and finally distilling under essentially non-cracking conditions in vacuum distillation zone 19 either with or without further addition of ammonia.

The sequence of steps illustrated in Fig. 1 may be considered the preferred manner of practicing the invention. When the process is practiced according to Fig. 2 or Fig. 3, the presence of caustic soda in the crude during the primary distillation is apt to cause difficulty due to plugging of tubes when conventional refinery tube stills are used in such topping operation. This difficulty is avoided when the process is practiced according to Fig. 1.

The following example illustrates the process

more specifically according to the embodiment of Fig. 1:

#### Example I

5 A mixture of Gulf Coastal crudes was subjected to a preliminary distillation to remove gasoline, kerosene and light gas oil hydrocarbons and to yield a mazout having an A. P. I. gravity of about 21 and an initial A. S. T. M. boiling point of about 550° F. A batch of the mazout was blown with ammonia gas at room temperature for 15 minutes, resulting in an ammonia content of roughly 0.3 lb. NH<sub>3</sub> per bbl. Aqueous caustic soda (38° Bé.) was then introduced into and mixed with the mazout in amount equivalent to 1.55 lbs. NaOH per bbl. The resulting mixture was vacuum distilled and several cuts of distillate were obtained. The cuts had a greenish bloom and bright appearance. Three fractions, designated A, B and C and having S. U. viscosities at 210° F. of about 45, 50 and 85 respectively, were subjected to color stability tests by heating to 105° C. and maintaining them at such temperature and exposed to the atmosphere for 16 hours. The initial and final N. P. A. colors are recorded below:

|                      | Cut A | Cut B | Cut C |
|----------------------|-------|-------|-------|
| Initial color.....   | 1 1/2 | 1 1/2 | 2 1/4 |
| Final color.....     | 1 1/2 | 2     | 2 1/2 |
| Change in color..... | 1/4   | 1/4   | 1/4   |

35 By way of comparison another batch of the mazout was treated in the same manner except that in this case no ammonia was used. Comparative results for similar cuts are as follows:

|                      | Cut A' | Cut B' | Cut C' |
|----------------------|--------|--------|--------|
| Initial color.....   | 1 1/4  | 2      | 2 1/4  |
| Final color.....     | 2      | 2 1/2  | 4 1/2  |
| Change in color..... | 1/4    | 1/2    | 1 1/2  |

45 Comparison of these data shows that the ammonia treatment resulted in improvement in both the initial color and color stability. The effect is particularly evident with respect to the heaviest distillate fraction. The distillates from the last mentioned run had a bluish bloom and darker appearance than those prepared by using ammonia.

50 The following example illustrates the substantial ineffectiveness of treating with caustic soda and ammonia when the amount of caustic soda used is below 1.2 lbs. NaOH per bbl. of mazout.

#### Example II

60 Another batch of the mazout used in Example I was blown with ammonia gas at room temperature for 15 minutes, after which the ammonia content of the mazout was roughly 0.3 lb. NH<sub>3</sub> per bbl. Aqueous caustic soda (38° Bé.) was then mixed with the mazout in amount equivalent to 1.16 lbs. NaOH per bbl. The mixture was vacuum distilled and cuts were taken similar to those in Example I. The cuts had a somewhat greenish bloom but did not have as bright appearance as the corresponding cuts of Example I. Color stability tests in this instance were made by maintaining the cuts, exposed to the atmosphere, at a temperature of 71° C. for 96 hours.

The initial and final N. P. A. colors were as follows:

|                 | Cut A          | Cut B          | Cut C            |
|-----------------|----------------|----------------|------------------|
| Initial color   | $1\frac{3}{4}$ |                |                  |
| Final color     | $2\frac{1}{4}$ | $2\frac{1}{2}$ | $3 -$            |
| Change in color | $\frac{1}{2}$  | $1$            | $1\frac{3}{4} +$ |

For purpose of comparison another batch of the same mazout was treated in similar manner except that no ammonia was used. Comparative results for similar cuts are as follows:

|                 | Cut A'           | Cut B'           | Cut C'           |
|-----------------|------------------|------------------|------------------|
| Initial color   | $1\frac{3}{4} +$ |                  |                  |
| Final color     | $2\frac{1}{2} +$ | $2\frac{1}{2} -$ | $3\frac{1}{4}$   |
| Change in color | $\frac{3}{4}$    | $\frac{3}{4} +$  | $1\frac{1}{4} +$ |

The foregoing data indicate that while the use of ammonia apparently caused some improvement in initial color, it did not effect consistent improvement in color stability. In fact, the ammonia appears to have had an adverse effect on color stability of the lightest and heaviest cuts even though the amount of ammonia used was approximately the same as in Example I. This illustrates the importance of employing a sufficient amount of caustic soda in practicing the invention.

Where the term "naphthenic base crude" is used herein, it should be understood to refer to crude petroleums having viscosity-gravity constants of about 0.86 or higher.

We claim:

1. In a process for preparing lubricating oil from naphthenic base crude petroleum wherein hydrocarbons boiling below the lubricating oil range are removed as distillate in a primary distillation step and lubricating oil is removed as distillate in a subsequent vacuum distillation step, the steps for producing lubricating oil having improved bloom and color stability characteristics which consist of reacting the charge to one of said distillation steps with ammonia in the presence of caustic soda, said ammonia and caustic soda having been added in amounts of at least 1.2 lbs. NaOH and 0.1 lb. NH<sub>3</sub>, respectively, per bbl. of mazout resulting from said first distillation step.

2. In a process for preparing lubricating oil which comprises distilling naphthenic base crude petroleum to remove hydrocarbons boiling below the lubricating oil range and vacuum distilling the resulting mazout to yield a distillate lubricating oil, the step for producing lubricating

oil having improved bloom and color stability characteristics which consists of reacting the mazout prior to said vacuum distillation with caustic soda and with ammonia in amounts of at least 1.2 lbs. NaOH and 0.1 lb. NH<sub>3</sub>, respectively, per bbl. of mazout.

3. In a process for preparing lubricating oil from naphthenic base crude petroleum wherein hydrocarbons boiling below the lubricating oil range are removed as distillate in a primary distillation step and lubricating oil is removed as distillate in a subsequent vacuum distillation step, the step for producing lubricating oil having improved bloom and color stability characteristics which consists of reacting the crude petroleum prior to said first distillation step with ammonia and caustic soda in amounts of at least 1.2 lbs. NaOH and 0.1 lb. NH<sub>3</sub>, respectively, per bbl. of mazout resulting from said first distillation step.

4. In a process for preparing lubricating oil from naphthenic base crude petroleum wherein hydrocarbons boiling below the lubricating oil range are removed as distillate in a primary distillation step and lubricating oil is removed as distillate in a subsequent vacuum distillation step, the steps for producing lubricating oil having improved bloom and color stability characteristics which consist of reacting the crude petroleum prior to said primary distillation step with caustic soda in amount of at least 1.2 lbs. NaOH per bbl. of mazout resulting from said primary distillation step and subsequently reacting the mazout prior to said vacuum distillation step with ammonia in amount of at least 0.1 lb. NH<sub>3</sub> per bbl. of mazout.

GEORGE E. REESE.  
JOHN L. LARKIN.

References Cited in the file of this patent  
UNITED STATES PATENTS

| Number    | Name          | Date          |
|-----------|---------------|---------------|
| 1,521,282 | Diggs         | Dec. 30, 1924 |
| 1,833,691 | Pew           | Nov. 24, 1931 |
| 2,002,747 | Morrell       | May 28, 1935  |
| 2,106,976 | Harris et al. | Feb. 1, 1938  |
| 2,187,883 | Lemmon        | Jan. 23, 1940 |
| 2,193,417 | Gage          | Mar. 12, 1940 |
| 2,352,064 | Zerbe         | June 20, 1944 |

FOREIGN PATENTS

| Number  | Country       | Date          |
|---------|---------------|---------------|
| 590,635 | Great Britain | July 24, 1947 |